



US008258444B2

(12) **United States Patent**  
**Ohtani et al.**

(10) **Patent No.:** **US 8,258,444 B2**  
(b5) **Date of Patent:** **Sep. 4, 2012**

(54) **FRONT COVER FOR VEHICLE LIGHTING FIXTURE, METHOD OF MANUFACTURING THE FRONT COVER, AND ELECTRIC HEATING STRUCTURE**

(75) Inventors: **Sumio Ohtani**, Minami-ashigara (JP); **Tadashi Kuriki**, Minami-ashigara (JP)

(73) Assignee: **Fujifilm Corporation**, Tokyo (JP)

(\*) Notice: Subject to any disclaimer, the term of this patent is extended or adjusted under 35 U.S.C. 154(b) by 197 days.

(21) Appl. No.: **12/937,446**

(22) PCT Filed: **Apr. 10, 2009**

(86) PCT No.: **PCT/JP2009/057400**

§ 371 (c)(1),  
(2), (4) Date: **Oct. 12, 2010**

(87) PCT Pub. No.: **WO2009/125854**

PCT Pub. Date: **Oct. 15, 2009**

(65) **Prior Publication Data**

US 2011/0044065 A1 Feb. 24, 2011

(30) **Foreign Application Priority Data**

Apr. 11, 2008 (JP) ..... 2008-103265

(51) **Int. Cl.**  
**H05B 3/10** (2006.01)

(52) **U.S. Cl.** ..... **219/552; 362/92; 362/293; 362/509; 264/272.11**

(58) **Field of Classification Search** ..... **362/487, 362/509, 293, 317, 335, 336, 92; 219/202, 219/220, 522, 552; 427/108, 118, 162; 264/272.11**

See application file for complete search history.

(56)

**References Cited**

**U.S. PATENT DOCUMENTS**

|                   |        |                       |         |
|-------------------|--------|-----------------------|---------|
| 1,923,970 A *     | 8/1933 | Dowling .....         | 362/376 |
| 4,728,775 A *     | 3/1988 | Van Straten .....     | 219/202 |
| 6,563,086 B1 *    | 5/2003 | Meirndorf et al. .... | 219/220 |
| 7,410,267 B2 *    | 8/2008 | Mochizuki .....       | 362/92  |
| 7,553,053 B2 *    | 6/2009 | Mochizuki .....       | 362/509 |
| 2006/0050521 A1 * | 3/2006 | Mochizuki .....       | 362/459 |

**FOREIGN PATENT DOCUMENTS**

|                |         |
|----------------|---------|
| JP 04-229983   | 8/1992  |
| JP 04-334891   | 11/1992 |
| JP 05-205859   | 8/1993  |
| JP 10-289602   | 10/1998 |
| JP 2007-026989 | 2/2007  |
| JP 2007-242290 | 9/2007  |
| JP 2007-242292 | 9/2007  |
| JP 2007-305338 | 11/2007 |

**OTHER PUBLICATIONS**

International Serach Report, PCT/JP2009/057400, May 12, 2009.

\* cited by examiner

*Primary Examiner* — John A Ward

(74) *Attorney, Agent, or Firm* — Young & Thompson

(57) **ABSTRACT**

A front cover for a vehicle lighting fixture is attached to the front opening part of the vehicle lighting fixture having a lamp body and a light source installed in the lamp body. A part of the surface of the front cover opposed to the light source includes a heating element having a three-dimensional curved surface. The heating element includes a mesh pattern having intersections of a large number of grids formed of conductive metallic filaments and a first electrode and a second electrode formed at both opposed ends of the mesh pattern. The projection shape of the outline of the entire mesh pattern is formed in a rectangular shape having the longitudinal direction, for example, between the first electrode and the second electrode.

**14 Claims, 23 Drawing Sheets**



FIG. 1



FIG. 2



FIG. 3A



FIG. 3B



FIG. 3C



FIG. 4



FIG. 5



FIG. 6A



FIG. 6B



FIG. 7



FIG. 8



FIG. 9



FIG. 10



FIG. 11



FIG. 12



FIG. 13



FIG. 14



RESIN INJECTION

FIG. 15A



FIG. 15B



FIG. 15C



FIG. 15D



FIG. 15E



FIG. 16A



FIG. 16B



FIG. 17A



FIG. 17B



FIG. 18



FIG. 19



FIG. 20



FIG. 21



FIG. 22



FIG. 23



## 1

**FRONT COVER FOR VEHICLE LIGHTING  
FIXTURE, METHOD OF MANUFACTURING  
THE FRONT COVER, AND ELECTRIC  
HEATING STRUCTURE**

**TECHNICAL FIELD**

The present invention relates to a car light front cover containing a transparent heat generator excellent in visibility and heat generation, a method for producing the front cover, and an electric heating structure containing the heat generator for various applications.

**BACKGROUND ART**

In general, illuminance of a car light may be reduced due to the following causes:

- (1) adhesion and accumulation of snow on the outer circumferential surface of the front cover,
- (2) adhesion and freezing of rain water or car wash water on the outer circumferential surface of the front cover, and
- (3) progression of (1) and (2) due to use of an HID lamp light source having a high light intensity even under a low power consumption (a small heat generation amount).

Structures described in Japanese Laid-Open Patent Publication Nos. 2007-026989 and 10-289602 have been proposed in view of preventing the above illuminance reduction of the car light.

The structure described in Japanese Laid-Open Patent Publication No. 2007-026989 is obtained by printing a conductive pattern on a transparent insulating sheet and by attaching the sheet to a formed lens using an in-mold method. Specifically, the conductive pattern is composed of a composition containing a noble metal powder and a solvent-soluble thermoplastic resin.

The structure described in Japanese Laid-Open Patent Publication No. 10-289602 is obtained by attaching a heat generator into a lens portion of a car lamp. The lens portion is heated by applying an electric power to the heat generator under a predetermined condition. Japanese Laid-Open Patent Publication No. 10-289602 describes that the heat generator comprises a transparent conductive film of ITO (Indium Tin Oxide), etc.

**DISCLOSURE OF THE INVENTION**

However, in the structure described in Japanese Laid-Open Patent Publication No. 2007-026989, the conductive pattern has a large width of 50 to 500  $\mu\text{m}$ . Particularly, a printed conductive wire having a width of 0.3 mm is used in the conductive pattern in Examples of Japanese Laid-Open Patent Publication No. 2007-026989. Such a thick conductive wire is visible to the naked eye, and the structure is disadvantageous in transparency.

In the case of using the thick conductive wire on a front cover of a headlamp, one wire may be arranged in a zigzag manner, thereby forming a long conductive line to obtain a desired resistance value (e.g. about 40 ohm). However, a potential difference may be disadvantageously generated between adjacent conductive line portions to cause migration.

On the other hand, the structure described in Japanese Laid-Open Patent Publication No. 10-289602 utilizes the transparent conductive film of ITO, etc. as the heat generator. The film cannot be formed on a curved surface of a front cover by a method other than vacuum sputtering methods. Thus, the structure is disadvantageous in efficiency, cost, etc.

## 2

In addition, since the transparent conductive film is composed of a ceramic such as ITO, the film is often cracked when a sheet on which the transparent conductive film is formed is bent in an in-mold method. Therefore, such a car light front cover having the curved-surface body and the transparent heater cannot be inexpensively produced and practically used.

In view of the above problems, an object of the present invention is to provide a car light front cover, a method for producing the front cover, and an electric heating structure, capable of forming a substantially transparent surface heat generation film on a curved surface, improving the heat generation uniformity, preventing the migration, and forming a transparent heater on a curved-surface body inexpensively.

10 The above object of the present invention is achieved by the following car light front cover, method for producing the front cover, and electric heating structure.

[1] A car light front cover according to a first aspect of the present invention, which is attached to a front opening of a car light having a lamp body and a light source disposed therein, wherein the front cover comprises a heat generator having a three-dimensional curved surface disposed in a part facing the light source, and the heat generator has a mesh pattern containing a conductive thin metal wire with a plurality of lattice intersections and further has first and second electrodes formed on the opposite ends of the mesh pattern.

[2] A car light front cover according to [1], wherein the thin metal wire in the mesh pattern has a width of 1 to 40  $\mu\text{m}$ .

[3] A car light front cover according to [1] or [2], wherein the thin metal wire in the mesh pattern has a pitch of 0.1 to 50 mm.

[4] A car light front cover according to any one of [1] to [3], wherein when two opposite points in the first and second electrodes are at a distance,  $L_{\min}$  is a minimum value of the distance, and  $L_{\max}$  is a maximum value of the distance, the first and second electrodes satisfy the inequality:

$$(L_{\max}-L_{\min})/((L_{\max}+L_{\min})/2) \leq 0.375.$$

[5] A car light front cover according to any one of [1] to [4], 40 wherein the thin metal wire in the mesh pattern has a metallic silver portion formed by exposing and developing a silver salt-containing layer containing a silver halide.

[6] A car light front cover according to any one of [1] to [4], wherein the thin metal wire in the mesh pattern has a patterned, plated metal layer.

[7] A car light front cover according to any one of [1] to [4], wherein the thin metal wire in the mesh pattern has a print of a metal powder paste.

[8] A car light front cover according to any one of [1] to [4], 50 wherein the thin metal wire in the mesh pattern has a copper foil patterned by etching.

[9] A car light front cover according to any one of [1] to [8], wherein the heat generator has a surface resistance of 10 to 500 ohm/sq.

[10] A car light front cover according to any one of [1] to [9], wherein the heat generator has an electrical resistance of 12 to 120 ohm.

[11] A car light front cover according to any one of [1] to [10], wherein the three-dimensional curved surface of the heat generator has a minimum curvature radius of 300 mm or less.

[12] A method according to a second aspect of the present invention for producing a car light front cover, which is attached to a front opening of a car light having a lamp body and a light source disposed therein, wherein the front cover comprises a heat generator disposed in a part facing the light source, the method comprises a heat generator preparation

process of preparing the heat generator and an injection process of placing the heat generator in a mold and then injecting a melted resin into the mold, and the heat generator preparation process contains a pattern formation step of forming a mesh pattern containing a conductive thin metal wire with a plurality of lattice intersections on an insulating transparent film, a shape forming step of forming the transparent film into a three-dimensional curved surface corresponding to the surface shape of the car light front cover, an electrode formation step of forming a first and second electrodes on the opposite ends of the transparent film, and a cutting step of cutting a part of the transparent film having the three-dimensional curved surface. The electrode formation step may be carried out after the cutting step.

[13] A method according to [12], wherein the thin metal wire formed in the pattern formation step has a width of 1 to 40  $\mu\text{m}$ .

[14] A method according to [12] or [13], wherein the thin metal wire in the mesh pattern formed in the pattern formation step has a pitch of 0.1 to 50 mm.

[15] A method according to any one of [12] to [14], wherein the first and second electrodes are formed in the electrode formation step such that when two opposite points in the first and second electrodes are at a distance,  $L_{\min}$  is a minimum value of the distance, and  $L_{\max}$  is a maximum value of the distance, the first and second electrodes satisfy the inequality:

$$(L_{\max} - L_{\min}) / ((L_{\max} + L_{\min}) / 2) \leq 0.375.$$

[16] A method according to any one of [12] to [15], wherein the mesh pattern containing the thin metal wire is formed on the transparent film in the pattern formation step such that the thin metal wire has a metallic silver portion formed by exposing and developing a silver salt-containing layer containing a silver halide.

[17] A method according to any one of [12] to [15], wherein the mesh pattern containing the thin metal wire is formed on the transparent film in the pattern formation step such that the thin metal wire has a patterned, plated metal layer.

[18] A method according to any one of [12] to [15], wherein the mesh pattern containing the thin metal wire is formed on the transparent film in the pattern formation step such that the thin metal wire has a print of a metal powder paste.

[19] A method according to any one of [12] to [15], wherein the mesh pattern containing the thin metal wire is formed on the transparent film in the pattern formation step such that the thin metal wire has a copper foil patterned by etching.

[20] A method according to any one of [12] to [19], wherein the heat generator has a surface resistance of 10 to 500 ohm/sq.

[21] A method according to any one of [12] to [20], wherein the heat generator has an electrical resistance of 12 to 120 ohm.

[22] A method according to any one of [12] to [21], wherein the heat generator has a three-dimensional curved surface with a minimum curvature radius of 300 mm or less.

[23] An electric heating structure according to a third aspect of the present invention, comprising a heat generator having a three-dimensional curved surface, wherein the heat generator has a mesh pattern containing a conductive thin metal wire with a plurality of lattice intersections and further has first and second electrodes formed on the opposite ends of the mesh pattern.

#### ADVANTAGEOUS EFFECTS OF INVENTION

As described above, in the car light front cover and the front cover production method of the present invention, a substan-

tially transparent surface heat generation film can be formed on a curved surface, the heat generation uniformity can be improved, the migration can be prevented, and a transparent heater can be inexpensively formed on a curved-surface body.

#### BRIEF DESCRIPTION OF DRAWINGS

FIG. 1 is a cross-sectional view partially showing a usage of a front cover according to an embodiment of the present invention;

FIG. 2 is a perspective view showing a heat generator according to the embodiment;

FIGS. 3A to 3C are each an explanatory view showing an overall projected shape of a mesh pattern;

FIG. 4 is an explanatory view showing a distance between two opposite points in first and second electrodes;

FIG. 5 is a perspective view showing the mesh pattern formed on a transparent film;

FIG. 6A is a cross-sectional view partially showing a forming mold for vacuum shape forming of the transparent film, and FIG. 6B is a cross-sectional view showing the transparent film pressed to the mold;

FIG. 7 is a perspective view showing the transparent film having a curved surface shape formed using the forming mold under vacuum;

FIG. 8 is a view showing the first and second electrodes formed on the transparent film having the curved surface shape in production of a heat generator according to a first specific example;

FIG. 9 is a perspective view showing the heat generator of the first specific example prepared by partially cutting the transparent film having the curved surface shape;

FIG. 10 is a view showing the first and second electrodes formed on the transparent film having the curved surface shape after partially cutting the film in production of a heat generator according to a second specific example;

FIG. 11 is a perspective view showing the prepared heat generator of the second specific example;

FIG. 12 is a view showing the first and second electrodes formed on the transparent film having the curved surface shape after partially cutting the film in production of a heat generator according to a third specific example;

FIG. 13 is a perspective view showing the prepared heat generator of the third specific example;

FIG. 14 is a cross-sectional view partially showing the heat generator of the embodiment placed in an injection mold;

FIGS. 15A to 15E are views showing the process of a method for forming the mesh pattern of the embodiment (a first method);

FIGS. 16A and 16B are views showing the process of another method for forming the mesh pattern of the embodiment (a second method);

FIGS. 17A and 17B are views showing the process of a further method for forming the mesh pattern of the embodiment (a third method);

FIG. 18 is a view showing the process of a still further method for forming the mesh pattern of the embodiment (a fourth method);

FIG. 19 is a plan view showing a front cover according to Example 1;

FIG. 20 is a plan view showing a front cover according to Reference Example 1;

FIG. 21 is a chart showing a temperature distribution of a heat generator according to Example 1;

FIG. 22 is a chart showing a temperature distribution of a heat generator according to Reference Example 1; and

FIG. 23 is a plan view showing first and second electrodes formed on a transparent film having a curved surface shape in production of front covers according to Examples 2 to 5 and Reference Example 2.

#### BEST MODE FOR CARRYING OUT THE INVENTION

An embodiment of the car light front cover and the front cover production method of the present invention will be described below with reference to FIGS. 1 to 23.

As shown in FIG. 1 omitted in part, a car light front cover 10 according to the embodiment (hereinafter referred to as the front cover 10) is attached to a front opening of a car light 16 having a lamp body 12 and a light source 14 disposed therein. The front cover 10 has a cover body 18 composed of a polycarbonate resin or the like and thereon a heat generator 20 (hereinafter referred to also as the transparent heat generator 20). The heat generator 20 has a curved surface shape, and is disposed on the surface facing the light source 14.

As shown in FIG. 2, the heat generator 20 has a mesh pattern 24 containing conductive thin metal wires 22 with a large number of lattice intersections (partially shown), and further has a first electrode 26 and a second electrode 28 formed on the opposite ends of the mesh pattern 24.

In this embodiment, the overall shape of the mesh pattern 24 may be different from the shape of the front cover 10. For example, as shown in FIG. 2, the projected shape 30 (the shape projected on the opening surface of the front cover 10) of the overall shape of the mesh pattern 24 may be preferably a rectangular shape having long sides between the first electrode 26 and the second electrode 28. Alternatively, as shown in FIG. 3A, the projected shape 30 may be preferably a rectangular shape having curved portions 32 protruding from the long sides integrally. It is to be understood that as shown in FIGS. 3B and 3C, the projected shape 30 may be a track or ellipsoid shape. As shown in FIG. 2, a region contained in the overall shape of the mesh pattern 24 acts as a heat generation region 34 of the heat generator 20.

In this embodiment, when two opposite points in the first electrode 26 and the second electrode 28 are at a distance, Lmin is a minimum value of the distance, and Lmax is a maximum value of the distance, the first electrode 26 and the second electrode 28 satisfy the inequality:

$$(L_{\max} - L_{\min}) / ((L_{\max} + L_{\min}) / 2) \leq 0.375.$$

The two opposite points in the first electrode 26 and the second electrode 28 are two points that are line-symmetric with respect to an imaginary centerline between the first electrode 26 and the second electrode 28. As shown in FIG. 4, the imaginary centerline is a line N perpendicular to a line Mj between the longitudinal middle point T1j in the first electrode 26 and the longitudinal middle point T2j in the second electrode 28. For example, the two opposite points include the longitudinal middle point T1j in the first electrode 26 and the longitudinal middle point T2j in the second electrode 28, and include the longitudinal end point T1n in the first electrode 26 and the longitudinal end point T2n in the second electrode 28. Furthermore, as shown in FIG. 4, the two opposite points include points T1<sub>1</sub> and T2<sub>1</sub>, points T1<sub>2</sub> and T2<sub>2</sub>, points T1<sub>3</sub> and T2<sub>3</sub>, etc. The minimum value Lmin is the shortest distance between such two opposite points, and the maximum value Lmax is the longest distance between such two opposite points. For example, when the projected shape 30 of the mesh pattern 24 is not a rectangular shape but a circular shape corresponding to the shape of the front cover 10 (shown by a two-dot chain line m), the maximum value Lmax is the dis-

tance between the points T1<sub>1</sub> and T2<sub>1</sub> shown by a two-dot chain line k along the circular shape, and the minimum value Lmin is the shortest distance between the middle points T1j and T2j.

5 The finding of the above relation between the minimum value Lmin and the maximum value Lmax and the realization of uniform heat generation in the heat generator formed on a particular position of a three-dimensional curved surface will be described below.

10 In conventional surface heat generators for rear windows and headlamp covers, a heat generation wire is distributed on the entire surface to be heated. In general, one wire is used in a small heater of the headlamp cover, and at most ten wires are used in a large heater of the rear window. A current flows from one end to the other end of the wire. Therefore, when all the wires are composed of the same material and have the same width and thickness, the heat generation amount depends on the density of the wires. Thus, in the conventional heat generator, uniform heat generation can be achieved by forming 15 the wires at a constant density, regardless of the shape of the region to be heated.

20 However, the conventional heat generator is disadvantageous in that the heat generation wire is highly visible to the naked eye, resulting in illuminance reduction of the light source. Thus, in this embodiment, the mesh pattern 24 is formed to prepare the heat generator 20 with a high transparency. The transparent heat generator 20 having the mesh pattern 24 contains innumerable current pathways, and a current is concentrated in a pathway with a low resistance. Therefore, an idea is required to achieve uniform heat generation.

25 A method for achieving uniform heat generation in the transparent heat generator 20 (particularly formed on a three-dimensional curved surface) has been found as follows.

30 Thus, the heat generation region 34 is formed such that the projected shape 30 is an approximately rectangular shape, strip-shaped electrodes (the first electrode 26 and the second electrode 28) are disposed on the opposite sides, and a voltage is applied between the first electrode 26 and the second electrode 28 to flow a current. Though the projected shape 30 cannot be a precise rectangular shape on the three-dimensional curved surface, it is preferred that the projected shape 30 is made closer to the rectangular shape.

35 When the heat generation wire is arranged in a zigzag manner in the conventional heat generator, a potential difference is generated between the adjacent conductive lines to cause migration disadvantageously. In contrast, in this embodiment, the mesh pattern 24 with a large number of lattice intersections is formed by the conductive thin metal wires 22, so that the adjacent wires are intrinsically in the 40 short circuit condition, and the migration is never a problem.

45 The electrical resistance of the transparent heat generator 20 is increased in proportion to the distance between the first electrode 26 and the second electrode 28 facing each other. Under a constant voltage, the heat generation amount varies 50 in inverse proportion to the electrical resistance. In other words, the heat generation amount is reduced as the electrical resistance is increased. Thus, it is ideal to arrange the first electrode 26 and the second electrode 28 parallel to each other. In the case of heating a particular region on the three-dimensional curved surface, it is preferred that the distance Ln between the two opposite points in the first electrode 26 and the second electrode 28 is within a narrow distance range 55 in any position to uniformly heat the surface.

60 It is considered that the problem of snow or frost is caused mainly at an ambient temperature of  $-10^{\circ}\text{C}$ . to  $+3^{\circ}\text{C}$ . At  $-10^{\circ}\text{C}$ . or lower, the ambient air is almost free from moisture, and the snow is reduced as well as the frost. At  $3^{\circ}\text{C}$ . or higher, the

snow or frost is preferably melted. When the heat generator 20 has a heat generation distribution (variation) of 0, the surface temperature of the front cover 10 can be increased from  $-10^{\circ}\text{C}$ . to  $3^{\circ}\text{C}$ . by heating the surface by  $13^{\circ}\text{C}$ . on average. However, when the heat generator 20 has a heat generation distribution (variation) of plus or minus  $5^{\circ}\text{C}$ ., it is necessary to heat the surface by  $18^{\circ}\text{C}$ . on average (distributed between  $13^{\circ}\text{C}$ . and  $23^{\circ}\text{C}$ .). The minimum surface temperature of the front cover 10 cannot be increased to  $3^{\circ}\text{C}$ . or higher only by heating the surface by  $13^{\circ}\text{C}$ . on average. Thus, the heat generator 20 having a smaller heat generation distribution (variation) is more advantageous in energy saving.

The temperature increased by the transparent heat generator 20 (the temperature rise range) is preferably such that the minimum is  $13^{\circ}\text{C}$ ., the maximum is  $19^{\circ}\text{C}$ ., and the average is  $16^{\circ}\text{C}$ . In this case, the energy can be preferably reduced by  $2^{\circ}\text{C}$ . as compared with the above described example, resulting in energy saving. In this case, the temperature distribution ratio is  $(19^{\circ}\text{C}.-13^{\circ}\text{C})/16^{\circ}\text{C}=0.375$ . Since the heat generation amount approximately corresponds to the distribution of the distance between the two opposite points in the first electrode 26 and the second electrode 28, the equality of  $(L_{\max}-L_{\min})/(L_{\max}+L_{\min})/2=0.375$  is satisfied, wherein  $L_{\max}$  and  $L_{\min}$  represent a maximum value and a minimum value of the distance respectively.

When the average temperature increased by the transparent heat generator 20 is controlled at  $14.5^{\circ}\text{C}$ ., the maximum temperature  $T_{\max}$  is  $14.5-13+14.5=16$ , and the temperature distribution ratio is  $(16-13)/14.5=0.207$ . Therefore, the first electrode 26 and the second electrode 28 may be arranged such that the equality of  $(L_{\max}-L_{\min})/(L_{\max}+L_{\min})/2=0.207$  is satisfied. In this case, the energy can be preferably reduced by  $1.5^{\circ}\text{C}$ . as compared with the above example using the average temperature of  $16^{\circ}\text{C}$ ., thereby being further advantageous in energy saving.

The heat generator 20 preferably has a surface resistance of 10 to 500 ohm/sq. In addition, the heat generator 20 preferably has an electrical resistance of 12 to 120 ohm. In this case, the average temperature increased by the heat generator 20 can be controlled at  $16^{\circ}\text{C}$ .,  $14.5^{\circ}\text{C}$ ., etc., and the snow or the like attached to the front cover 10 can be removed.

In this embodiment, the thin metal wire 22 in the mesh pattern 24 preferably has a width of 1 to  $40\text{ }\mu\text{m}$ . In this case, because the mesh pattern 24 can be made less visible, the transparency increases. As a result, the illuminance reduction of the light source 14 is prevented.

The thin metal wire 22 in the mesh pattern 24 preferably has a pitch of 0.1 to 50 mm when the thin metal wire 22 has a width of 1 to  $40\text{ }\mu\text{m}$ , the heat generator 20 has a surface resistance of 10 to 500 ohm/sq, and the heat generator 20 has an electrical resistance of 12 to 120 ohm.

A method for producing the front cover 10 will be described below with reference to FIGS. 5 to 18.

First, as shown in FIG. 5, the mesh pattern 24 containing the conductive thin metal wires 22 with a large number of lattice intersections is formed on an insulating transparent film 40.

Then, as shown in FIG. 6A, the transparent film 40 having the mesh pattern 24 is formed under vacuum into a curved surface shape corresponding to the surface shape of the front cover 10. The vacuum forming is carried out using a forming mold 42 having approximately the same size as an injection mold 50 for injection forming of the front cover 10 (see FIG. 14). As shown in FIG. 6A, when the front cover 10 has a three-dimensional curved surface, the forming mold 42 has a similar curved surface (an inverted curved surface in this case) and a plurality of vacuum vents 44. For example, when

the front cover 10 has a concave curved surface, the forming mold 42 has such a size that a convex curved surface 46 thereof is fitted into the concave curved surface of the front cover 10.

5 The vacuum forming of the transparent film 40 may be carried out using the forming mold 42 as follows. As shown in FIG. 6A, the transparent film 40 having the mesh pattern 24 is preheated at  $140^{\circ}\text{C}$ . to  $210^{\circ}\text{C}$ . Then, as shown in FIG. 6B, the transparent film 40 is pressed to the convex curved surface 46 of the forming mold 42, and an air pressure of 0.1 to 2 MPa is applied to the transparent film 40 by vacuuming air through the vacuum vents 44 in the forming mold 42. As shown in FIG. 7, the transparent film 40 having the same curved surface shape as the front cover 10 is obtained by the vacuum forming.

As shown in FIG. 8, the first electrode 26 and the second electrode 28 are formed on predetermined positions in the transparent film 40 having the curved surface shape. For example, conductive first copper tapes 48a (for forming strip electrodes) are attached to the transparent film 40, and second copper tapes 48b (for forming lead-out electrodes) are arranged in the direction perpendicular to the first copper tapes 48a, to form the first electrode 26 and the second electrode 28. The second copper tapes 48b are partially overlapped with the first copper tapes 48a.

As shown in FIG. 9, a part of the transparent film 40 having the curved surface shape is cut off. For example, the cutting may be carried out such that the overall projected shape 30 of 30 the mesh pattern 24 in the transparent film 40 is converted to a rectangular shape while maintaining the first electrode 26 and the second electrode 28. In this embodiment, as shown in FIG. 8, the periphery of the transparent film 40 having the curved surface shape is cut along a cutting line L1 to obtain a 35 circular projected shape corresponding to the formed shape, and curved portions 41 at the ends are cut along cutting lines L2 and L3, while maintaining the first electrode 26 and the second electrode 28. Thus, as shown in FIG. 9, a heat generator 20A according to a first specific example is obtained.

40 It is to be understood that the first electrode 26 and the second electrode 28 may be formed after partially cutting the transparent film 40 having the curved surface shape.

For example, as shown in FIG. 10, the periphery of the transparent film 40 having the curved surface shape is cut along a cutting line L1 to obtain a circular projected shape corresponding to the formed shape, curved portions 41 at the ends are cut along cutting lines L2 and L3, conductive first copper tapes 48a (for forming strip electrodes) are attached onto the periphery of the transparent film 40, and second copper tapes 48b (for forming lead-out electrodes) are arranged in the direction perpendicular to the first copper tapes 48a to form the first electrode 26 and the second electrode 28. The second copper tapes 48b are partially overlapped with the first copper tapes 48a. Thus, as shown in FIG. 11, a heat generator 20B according to a second specific example is obtained.

60 Alternatively, for example, as shown in FIG. 12, the periphery of the transparent film 40 having the curved surface shape is cut along a cutting line L4 to obtain a circular projected shape with a flat surface portion, curved portions at the ends are cut along cutting lines L2 and L3, conductive first copper tapes 48a (for forming strip electrodes) are attached to the periphery of the flat surface portion in the transparent film 40, and second copper tapes 48b (for forming lead-out electrodes) are arranged in the direction perpendicular to the first copper tapes 48a to form the first electrode 26 and the second electrode 28. The second copper tapes 48b are partially over-

lapped with the first copper tapes **48a**. Thus, as shown in FIG. 13, a heat generator **20C** according to a third specific example is obtained.

The heat generator **20** shown in FIG. 2 and the heat generators **20A** to **20C** of the first to third specific examples are hereinafter referred to as the heat generator **20**.

As shown in FIG. 14, the heat generator **20** obtained in the above manner is placed in the injection mold **50** for forming the front cover **10**.

A melted resin is introduced into a cavity **52** of the injection mold **50**, and is hardened therein to obtain the front cover **10** having the integrated heat generator **20**.

Several methods (first to fourth methods) for forming the mesh pattern **24** containing the thin metal wires **22** on the transparent film **40** will be described below with reference to FIGS. 15A to 18.

In the first method, a photosensitive silver salt layer is formed, exposed, developed, and fixed on the transparent film **40**, to form metallic silver portions in the mesh pattern.

Specifically, as shown in FIG. 15A, the transparent film **40** is coated with a photosensitive silver salt layer **58** containing a mixture of a gelatin **56** and a silver halide **54** (e.g., silver bromide particles, silver chlorobromide particles, or silver iodobromide particles). Though the silver halide **54** is exaggeratedly shown by points in FIGS. 15A to 15C to facilitate understanding, the points do not represent the size, concentration, etc. of the silver halide **54**.

Then, as shown in FIG. 15B, the photosensitive silver salt layer **58** is subjected to an exposure treatment for forming the mesh pattern **24**. When an optical energy is applied to the silver halide **54**, minute silver nuclei are generated to form an invisible latent image.

As shown in FIG. 15C, the photosensitive silver salt layer **58** is subjected to a development treatment for converting the latent image to an image visible to the naked eye. Specifically, the photosensitive silver salt layer **58** having the latent image is developed using a developer, which is an alkaline or acidic solution, generally an alkaline solution. In the development treatment, using the latent image silver nuclei as catalyst cores, silver ions from the silver halide particles or the developer are reduced to metallic silver by a reducing agent (a developing agent) in the developer. As a result, the latent image silver nuclei are grown to form a visible silver image (developed silvers **60**).

The photosensitive silver halide **54** remains in the photosensitive silver salt layer **58** after the development treatment. As shown in FIG. 15D, the silver halide **54** is removed by a fixation treatment using a fixer, which is an acidic or alkaline solution, generally an acidic solution.

After the fixation treatment, metallic silver portions **62** are formed in exposed areas, and light-transmitting portions **64** containing only the gelatin **56** are formed in unexposed areas. Thus, the mesh pattern **24** is formed by the combination of the metallic silver portions **62** and the light-transmitting portions **64** on the transparent film **40**.

In a case where silver bromide is used as the silver halide **54** and a thiosulfate salt is used in the fixation treatment, a reaction represented by the following formula proceeds in the treatment.



Two thiosulfate  $\text{S}_2\text{O}_3$  ions and one silver ion in the gelatin **56** (from  $\text{AgBr}$ ) are reacted to generate a silver thiosulfate complex. The silver thiosulfate complex has a high water solubility, and thereby is eluted from the gelatin **56**. As a

result, the developed silvers **60** are fixed as the metallic silver portions **62**. The mesh pattern **24** is formed by the metallic silver portions **62**.

Thus, the latent image is reacted with the reducing agent to deposit the developed silvers **60** in the development treatment, and the residual silver halide **54**, not converted to the developed silver **60**, is eluted into water in the fixation treatment. The treatments are described in detail in T. H. James, "The Theory of the Photographic Process, 4th ed.", Macmillan Publishing Co., Inc., NY, Chapter 15, pp. 438-442, 1977.

The development treatment is generally carried out using the alkaline solution. Therefore, the alkaline solution used in the development treatment may be mixed into the fixer (generally an acidic solution), whereby the activity of the fixer may be disadvantageously changed in the fixation treatment. Further, the developer may remain on the film after removing the film from the development bath, whereby an undesired development reaction may be accelerated by the developer. Thus, it is preferred that the photosensitive silver salt layer **58** is neutralized or acidified by a quencher such as an acetic acid solution after the development treatment before the fixation treatment.

For example, as shown in FIG. 15E, a conductive metal layer **66** may be disposed only on the metallic silver portion **62** by a plating treatment (such as an electroless plating treatment, an electroplating treatment, or a combination thereof). In this case, the mesh pattern **24** is formed by the metallic silver portions **62** and the conductive metal layers **66** disposed thereon.

In the second method, for example, as shown in FIG. 16A, a photoresist film **70** is formed on a copper foil **68** disposed on the transparent film **40**, and the photoresist film **70** is exposed and developed to form a resist pattern **72**. As shown in FIG. 16B, the copper foil **68** exposed from the resist pattern **72** is etched to form the mesh pattern **24** of the copper foil **68**.

In the third method, as shown in FIG. 17A, a paste **74** containing fine metal particles is printed on the transparent film **40** to form the mesh pattern **24**. Of course, as shown in FIG. 17B, the printed paste **74** may be plated with a metal to form a plated metal layer **76**. In this case, the mesh pattern **24** is formed by the paste **74** and the plated metal layer **76**.

In the fourth method, as shown in FIG. 18, a thin metal film **78** is printed on the transparent film **40** to form the mesh pattern by using a screen or gravure printing plate.

Among the first to fourth methods, suitable for preparing the heat generator **20** having the curved surface shape is the first method containing exposing, developing, and fixing the photosensitive silver salt layer **58** disposed on the transparent film **40** to form the mesh pattern **24** of the metallic silver portions **62**.

As described above, in the heat generator **20** and the front cover **10** equipped therewith according to the embodiment, the substantially transparent surface heat generation film can be formed on the curved surface, the heat generation uniformity can be improved, the migration can be prevented, and the transparent heater can be inexpensively formed on the curved surface of the formed body.

Though the heat generator **20** is formed in a part of the surface of the front cover **10** having the entirely curved surface shape in FIG. 1, the front cover **10** may have a partially curved shape and a flat surface. The mesh pattern **24** in the heat generator **20** of the embodiment can be flexibly used on such a partially curved shape. Furthermore, the mesh pattern **24** can be used on a curved surface shape having a minimum curvature radius of 300 mm or less. Thus, the mesh pattern **24** can be satisfactorily used on various curved surface shapes.

## 11

without breaking, even when the heat generator **20** has a curved surface shape with a minimum curvature radius of 300 mm or less.

A particularly preferred method, which contains using a photographic photosensitive silver halide material for forming the mesh pattern **24** in the heat generator **20** of this embodiment, will be mainly described below.

As described above, the mesh pattern **24** in the heat generator **20** of this embodiment may be prepared as follows. A photosensitive material having the transparent film **40** and thereon a photosensitive silver halide-containing emulsion layer is exposed and developed, whereby the metallic silver portions **62** and the light-transmitting portions **64** are formed in the exposed areas and the unexposed areas respectively. The metallic silver portions **62** may be subjected to a physical development treatment and/or a plating treatment to form the conductive metal layer **66** thereon if necessary.

The method for forming the mesh pattern **24** includes the following three processes, different in the photosensitive materials and development treatments.

(1) A process comprising subjecting a photosensitive black-and-white silver halide material free of physical development nuclei to a chemical or physical development, to form the metallic silver portions **62** on the material.

(2) A process comprising subjecting a photosensitive black-and-white silver halide material having a silver halide emulsion layer containing physical development nuclei to a physical development, to form the metallic silver portions **62** on the photosensitive material.

(3) A process comprising subjecting a stack of a photosensitive black-and-white silver halide material free of physical development nuclei and an image-receiving sheet having a non-photosensitive layer containing physical development nuclei to a diffusion transfer development, to form the metallic silver portions **62** on the non-photosensitive image-receiving sheet.

In the process of (1), an integral black-and-white development procedure is used to form a transmittable conductive film such as a light-transmitting electromagnetic-shielding film or a light-transmitting conductive film on the photosensitive material. The resulting silver is a chemically or physically developed silver containing a filament of a high-specific surface area, and shows a high activity in the following plating or physical development treatment.

In the process of (2), the silver halide particles are melted around the physical development nuclei and deposited on the nuclei in the exposed areas, to form a transmittable conductive film on the photosensitive material. Also in this process, an integral black-and-white development procedure is used. Though high activity can be achieved since the silver halide is deposited on the physical development nuclei in the development, the developed silver has a spherical shape with small specific surface.

In the process of (3), the silver halide particles are melted in unexposed areas, and diffused and deposited on the development nuclei of the image-receiving sheet, to form a transmittable conductive film on the sheet. In this process, a so-called separate-type procedure is used, and the image-receiving sheet is peeled off from the photosensitive material.

A negative development treatment or a reversal development treatment can be used in the processes. In the diffusion transfer development, the negative development treatment can be carried out using an auto-positive photosensitive material.

The chemical development, thermal development, solution physical development, and diffusion transfer development have the meanings generally known in the art, and are

## 12

explained in common photographic chemistry texts such as Shin-ichi Kikuchi, "Shashin Kagaku (Photographic Chemistry)", Kyoritsu Shuppan Co., Ltd., 1955 and C. E. K. Mees, "The Theory of Photographic Processes, 4th ed.", Mcmillan, 1977. A liquid treatment is generally used in the present invention, and also a thermal development treatment can be utilized. For example, techniques described in Japanese Laid-Open Patent Publication Nos. 2004-184693, 2004-334077, and 2005-010752 and Japanese Patent Application Nos. 10 2004-244080 and 2004-085655 can be used in the present invention.

(Photosensitive Material)

[Transparent Film **40**]

The transparent film **40** used in the production method of the embodiment may be a flexible plastic film.

Examples of materials for the plastic film include polyethylene terephthalates (PET), polyethylene naphthalates (PEN), polyvinyl chlorides, polyvinylidene chlorides, polyvinyl butyrls, polyamides, polyethers, polysulfones, polyether sulfones, polycarbonates, polyarylates, polyetherimides, polyetherketones, polyether ether ketones, polyolefins such as EVA, polycarbonates, triacetyl celluloses (TAC), acrylic resins, polyimides, and aramids.

In this embodiment, the polyethylene terephthalate is preferred as the material for the plastic film from the viewpoints of light transmittance, heat resistance, handling, and cost. The material may be appropriately selected depending on the requirement of heat resistance, heat plasticity, etc. An unstretched PET film is generally used for forming the curved surface shape. However, in the case of preparing the photosensitive material according to the present invention, a stretched PET film is used. The stretched PET film cannot be easily processed into the curved surface shape. Though the unstretched PET film can be processed at about 150°C., the processing temperature of the stretched PET film is preferably 170°C. to 250°C., more preferably 180°C. to 230°C.

The plastic film may have a monolayer structure or a multilayer structure containing two or more layers.

[Protective Layer]

In the photosensitive material, a protective layer may be formed on the emulsion layer to be hereinafter described. The protective layer used in this embodiment contains a binder such as a gelatin or a high-molecular polymer, and is formed on the photosensitive emulsion layer to improve the scratch prevention or mechanical property. In the case of performing the plating treatment, it is preferred that the protective layer is not formed or is formed with a small thickness. The thickness of the protective layer is preferably 0.2 μm or less. The method of applying or forming the protective layer is not particularly limited, and may be appropriately selected from known coating methods.

[Emulsion Layer]

The photosensitive material used in the production method of this embodiment preferably has the transparent film **40** and thereon the emulsion layer containing the silver salt as a light sensor (the silver salt-containing layer **58**). The emulsion layer according to the embodiment may contain a dye, a binder, a solvent, etc. in addition to the silver salt, if necessary.

<Silver Salt>

The silver salt used in this embodiment is preferably an inorganic silver salt such as a silver halide. It is particularly preferred that the silver salt is used in the form of particles for the photographic photosensitive silver halide material. The silver halide has an excellent light sensing property.

The silver halide, preferably used in the photographic emulsion of the photographic photosensitive silver halide material, will be described below.

In this embodiment, the silver halide is preferably used as a light sensor. Silver halide technologies for photographic silver salt films, photographic papers, print engraving films, emulsion masks for photomasking, and the like may be utilized in this embodiment.

The silver halide may contain a halogen element of chlorine, bromine, iodine, or fluorine, and may contain a combination of the elements. For example, the silver halide preferably contains  $\text{AgCl}$ ,  $\text{AgBr}$ , or  $\text{AgI}$ , more preferably contains  $\text{AgBr}$  or  $\text{AgCl}$ , as a main component. Also silver chlorobromide, silver iodochlorobromide, or silver iodo bromide is preferably used as the silver halide. The silver halide is further preferably silver chlorobromide, silver bromide, silver iodochlorobromide, or silver iodo bromide, most preferably silver chlorobromide or silver iodochlorobromide having a silver chloride content of 50 mol % or more.

The term "the silver halide contains  $\text{AgBr}$  (silver bromide) as a main component" means that the mole ratio of bromide ion is 50% or more in the silver halide composition. The silver halide particle containing  $\text{AgBr}$  as a main component may contain iodide or chloride ion in addition to the bromide ion.

The silver halide emulsion used in this embodiment may contain a metal of Group VIII or VIIB. It is particularly preferred that the emulsion contains a rhodium compound, an iridium compound, a ruthenium compound, an iron compound, an osmium compound, or the like to achieve four or more tones and low fogging.

The silver halide emulsion may be effectively doped with a hexacyano-metal complex such as  $\text{K}_4[\text{Fe}(\text{CN})_6]$ ,  $\text{K}_4[\text{Ru}(\text{CN})_6]$ , or  $\text{K}_3[\text{Cr}(\text{CN})_6]$  for increasing the sensitivity.

The amount of the compound added per 1 mol of the silver halide is preferably  $10^{-10}$  to  $10^{-2}$  mol/mol Ag, more preferably  $10^{-9}$  to  $10^{-3}$  mol/mol Ag.

Further, in this embodiment, the silver halide may preferably contain Pd (II) ion and/or Pd metal. Pd is preferably contained in the vicinity of the surface of the silver halide particle though it may be uniformly distributed therein. The term "Pd is contained in the vicinity of the surface of the silver halide particle" means that the particle has a layer with a higher palladium content in a region of 50 nm or less in the depth direction from the surface.

Such silver halide particle can be prepared by adding Pd during the particle formation. Pd is preferably added after the silver ion and halogen ion are respectively added by 50% or more of the total amounts. It is also preferred that Pd (II) ion is added in an after-ripening process to obtain the silver halide particle containing Pd near the surface.

The Pd-containing silver halide particle acts to accelerate the physical development and electroless plating, improve production efficiency of the desired heat generator, and lower the production cost. Pd is well known and used as an electroless plating catalyst. In the present invention, Pd can be located in the vicinity of the surface of the silver halide particle, so that the amount of the remarkably expensive Pd can be reduced.

In this embodiment, the content of the Pd ion and/or Pd metal per 1 mol of silver in the silver halide is preferably  $10^{-4}$  to 0.5 mol/mol Ag, more preferably 0.01 to 0.3 mol/mol Ag.

Examples of Pd compounds used include  $\text{PdCl}_4$  and  $\text{Na}_2\text{PdCl}_4$ .

In this embodiment, the sensitivity as the light sensor may be further increased by chemical sensitization, which is generally used for photographic emulsions. Examples of the chemical sensitization methods include chalcogen sensitization methods (such as sulfur, selenium, and tellurium sensitization methods), noble metal sensitization methods (such as gold sensitization methods), and reduction sensitization

methods. The methods may be used singly or in combination. Preferred combinations of the chemical sensitization methods include combinations of a sulfur sensitization method and a gold sensitization method, combinations of a sulfur sensitization method, a selenium sensitization method, and a gold sensitization method, and combinations of a sulfur sensitization method, a tellurium sensitization method, and a gold sensitization method.

<Binder>

10 The binder may be used in the emulsion layer to uniformly disperse the silver salt particles and to help the emulsion layer adhere to a support. In the present invention, the binder may contain a water-insoluble or water-soluble polymer, and preferably contains a water-soluble polymer.

15 Examples of the binders include gelatins, polyvinyl alcohols (PVA), polyvinyl pyrrolidones (PVP), polysaccharides such as starches, celluloses and derivatives thereof, polyethylene oxides, polysaccharides, polyvinylamines, chitosans, polylysines, polyacrylic acids, polyalginic acids, polyhyaluronic acids, and carboxycelluloses. The binders show a neutral, anionic, or cationic property depending on the ionicity of a functional group.

20 The amount of the binder in the emulsion layer is controlled preferably such that the Ag/binder volume ratio of the silver salt-containing layer is 1/4 or more, more preferably such that the Ag/binder volume ratio is 1/2 or more.

<Solvent>

25 The solvent used for forming the emulsion layer is not particularly limited, and examples thereof include water, organic solvents (e.g. alcohols such as methanol, ketones such as acetone, amides such as formamide, sulfoxides such as dimethyl sulfoxide, esters such as ethyl acetate, ethers), ionic liquids, and mixtures thereof.

30 In the present invention, the mass ratio of the solvent to the total of the silver salt, the binder, and the like in the emulsion layer is 30% to 90% by mass, preferably 50% to 80% by mass.

The treatments for forming the mesh pattern 24 will be described below.

[Exposure]

35 In this embodiment, the photosensitive material having the silver salt-containing layer 58 formed on the transparent film 40 is subjected to an exposure treatment. The exposure may be carried out using an electromagnetic wave. For example, a light (such as a visible light or an ultraviolet light) or a radiation ray (such as an X-ray) may be used to generate the electromagnetic wave. The exposure may be carried out using a light source having a wavelength distribution or a specific wavelength.

40 The exposure for forming a pattern image may be carried out using a surface exposure method or a scanning exposure method. In the surface exposure method, the photosensitive surface is irradiated with a uniform light through a mask to form an image of a mask pattern. In the scanning exposure method, the photosensitive surface is scanned with a beam of 45 a laser light or the like to form a patterned irradiated area.

45 In this embodiment, various laser beams can be used in the exposure. For example, a monochromatic high-density light of a gas laser, a light-emitting diode, a semiconductor laser, or a second harmonic generation (SHG) light source containing a nonlinear optical crystal in combination with a semiconductor laser or a solid laser using a semiconductor laser as an excitation source can be preferably used for the scanning exposure. Also a KrF excimer laser, an ArF excimer laser, an F2 laser, or the like can be used in the exposure. It is preferred 50 that the exposure is carried out using the semiconductor laser or the second harmonic generation (SHG) light source containing the nonlinear optical crystal in combination with the

## 15

semiconductor laser or the solid laser to reduce the size and costs of the system. It is particularly preferred that the exposure is carried out using the semiconductor laser from the viewpoints of reducing the size and costs and improving the durability and stability of the apparatus.

It is preferred that the silver salt-containing layer 58 is exposed in the pattern by the scanning exposure method using the laser beam. A capstan-type laser scanning exposure apparatus described in Japanese Laid-Open Patent Publication No. 2000-39677 is particularly preferably used for this exposure. In the capstan-type apparatus, a DMD described in Japanese Laid-Open Patent Publication No. 2004-1224 is preferably used instead of a rotary polygon mirror in the optical beam scanning system. Particularly in the case of producing a long flexible film heater having a length of 3 m or more, it is preferred that the photosensitive material is exposed to a laser beam on a curved exposure stage while conveying the material.

The structure of the mesh pattern 24 is not particularly limited as long as a current can flow between the electrodes under an applied voltage. The mesh pattern 24 may be a lattice pattern of triangle, quadrangle (e.g., rhombus, square), hexagon, etc. formed by crossing straight thin wires substantially parallel to each other. Furthermore, the mesh pattern 24 may be a pattern of straight, zigzag, or wavy wires parallel to each other.

[Development Treatment]

In this embodiment, the emulsion layer is subjected to a development treatment after the exposure. Common development treatment technologies for photographic silver salt films, photographic papers, print engraving films, emulsion masks for photomasking, and the like may be used in the present invention. A developer for the development treatment is not particularly limited, and may be a PQ developer, an MQ developer, an MAA developer, etc. Examples of commercially available developers usable in the present invention include CN-16, CR-56, CP45X, FD-3, and PAPITOL available from FUJIFILM Corporation, C-41, E-6, RA-4, D-19, and D-72 available from Eastman Kodak Company, and developers contained in kits thereof. The developer may be a lith developer.

Examples of the lith developers include D85 available from Eastman Kodak Company. In the present invention, by the exposure and development treatments, the metallic silver portion (preferably the patterned metallic silver portion) is formed in the exposed area, and the light-transmitting portion is formed in the unexposed area.

The developer for the development treatment may contain an image quality improver for improving the image quality. Examples of the image quality improvers include nitrogen-containing heterocyclic compounds such as benzotriazole. Particularly, a polyethylene glycol is preferably used for the lith developer.

The mass ratio of the metallic silver contained in the exposed area after the development to the silver contained in this area before the exposure is preferably 50% or more, more preferably 80% or more by mass. When the mass ratio is 50% by mass or more, a high conductivity can be achieved.

In this embodiment, the tone (gradation) obtained by the development is preferably more than 4.0, though not particularly restrictive. When the tone is more than 4.0 after the development, the conductivity of the conductive metal portion can be increased while maintaining high transmittance of the light-transmitting portion. For example, the tone of 4.0 or more can be achieved by doping with rhodium or iridium ion.

## 16

[Physical Development and Plating Treatment]

In this embodiment, to increase the conductivity of the metallic silver portion 62 formed by the exposure and development, conductive metal particles may be deposited thereon by a physical development treatment and/or a plating treatment. The conductive metal particles may be deposited on the metallic silver portion 62 by only one of the physical development and plating treatments or by the combination of the physical development and plating treatments.

10 In this embodiment, the physical development is such a process that metal ions such as silver ions are reduced by a reducing agent, whereby metal particles are deposited on nuclei of a metal or metal compound. Such physical development has been used in the fields of instant B & W film, instant slide film, printing plate production, etc., and the technologies can be used in the present invention.

15 The physical development may be carried out at the same time as the above development treatment after the exposure, and may be carried out after the development treatment separately.

20 The present invention may be appropriately combined with technologies described in the following patent publications: Japanese Laid-Open Patent Publication Nos. 2004-221564, 2004-221565, 2007-200922, and 2006-352073; International

25 Patent Publication No. 2006/001461; Japanese Laid-Open Patent Publication Nos. 2007-129205, 2008-251417, 2007-235115, 2007-207987, 2006-012935, 2006-010795, 2006-228469, 2006-332459, 2007-207987, and 2007-226215;

30 International Patent Publication No. 2006/088059; Japanese Laid-Open Patent Publication Nos. 2006-261315, 2007-072171, 2007-102200, 2006-228473, 2006-269795, 2006-267635, and 2006-267627; International Patent Publication No. 2006/098333; Japanese Laid-Open Patent Publication Nos. 2006-324203, 2006-228478, 2006-228836, and 2006-

35 228480; International Patent Publication Nos. 2006/098336 and 2006/098338; Japanese Laid-Open Patent Publication Nos. 2007-009326, 2006-336057, 2006-339287, 2006-336090, 2006-336099, 2007-039738, 2007-039739, 2007-039740, 2007-002296, 2007-084886, 2007-092146, 2007-

40 162118, 2007-200872, 2007-197809, 2007-270353, 2007-308761, 2006-286410, 2006-283133, 2006-283137, 2006-348351, 2007-270321, and 2007-270322; International Patent Publication No. 2006/098335; Japanese Laid-Open Patent Publication Nos. 2007-088218, 2007-201378, and 2007-335729; International Patent Publication No. 2006/098334; Japanese Laid-Open Patent Publication Nos. 2007-134439, 2007-149760, 2007-208133, 2007-178915, 2007-334325, 2007-310091, 2007-311646, 2007-013130, 2006-339526, 2007-116137, 2007-088219, 2007-207883, 2007-

45 207893, 2007-207910, and 2007-013130; International Patent Publication No. 2007/001008; Japanese Laid-Open Patent Publication Nos. 2005-302508 and 2005-197234.

50 The heat generator of the embodiment can be used in an electric heating structure for various applications (such as windows of vehicles, aircrafts, and buildings). Examples of the electric heating structures include electric heating windows of vehicles, aircrafts, buildings, etc.

EXAMPLES

60

First Example

65 The present invention will be described more specifically below with reference to Examples. Materials, amounts, ratios, treatment contents, treatment procedures, and the like, used in Examples, may be appropriately changed without departing from the scope of the present invention. The fol-

lowing specific examples are therefore to be considered in all respects as illustrative and not restrictive.

### Example 1

#### <Formation of Mesh Pattern 24 (Exposure and Development of Photosensitive Silver Salt Layer)>

An emulsion containing an aqueous medium, a gelatin, and silver iodobromide particles was prepared. The silver iodobromide particles had an I content of 2 mol % and an average spherical equivalent diameter of 0.05  $\mu\text{m}$ , and the amount of the gelatin was 7.5 g per 60 g of Ag (silver). The emulsion had an Ag/gelatin volume ratio of 1/1, and the gelatin had a low average molecular weight of 20000.

$\text{K}_3\text{Rh}_2\text{Br}_9$  and  $\text{K}_2\text{IrCl}_6$  were added to the emulsion at a concentration of  $10^{-7}$  mol/mol-silver to dope the silver bromide particles with Rh and Ir ions.  $\text{Na}_2\text{PdCl}_4$  was further added to the emulsion, and the resultant emulsion was subjected to gold-sulfur sensitization using chlorauric acid and sodium thiosulfate. The emulsion and a gelatin hardening agent were applied to a polyethylene terephthalate (PET) such that the amount of the applied silver was 1 g/m<sup>2</sup>. The PET was hydrophilized before the application. The coating was dried and exposed to an ultraviolet lamp using a photo-mask having a lattice-patterned space (line/space=285  $\mu\text{m}$ /15  $\mu\text{m}$  (pitch 300  $\mu\text{m}$ )), capable of forming a patterned developed silver image (line/space=15  $\mu\text{m}$ /285  $\mu\text{m}$ ). Then the coating was developed using the following developer at 25° C. for 45 seconds, fixed using the fixer SUPER FUJIFIX available from FUJIFILM Corporation, and rinsed with pure water. Thus obtained transparent film 40 having a mesh pattern 24 had a surface resistance of 40 ohm/sq.

#### [Developer Composition]

1 L of the developer contained the following compounds.

|                         |             |
|-------------------------|-------------|
| Hydroquinone            | 0.037 mol/L |
| N-methylaminophenol     | 0.016 mol/L |
| Sodium metaborate       | 0.140 mol/L |
| Sodium hydroxide        | 0.360 mol/L |
| Sodium bromide          | 0.031 mol/L |
| Potassium metabisulfite | 0.187 mol/L |

#### <Vacuum Forming>

The above transparent film 40 having the mesh pattern 24 was formed under vacuum using a forming mold 42 (see FIGS. 6A and 6B). The forming mold 42 had a diameter of 110 mm and a shape provided by cutting off a part of a sphere having a radius of 100 mm. In the vacuum forming, the transparent film 40 was preheated for 5 seconds by a hot plate at 195° C. and then immediately pressed onto the forming mold 42, and an air pressure of 0.7 MPa was applied to on the side of the transparent film 40 while vacuuming from the forming mold 42. Thus, the transparent film 40 was formed into an entirely curved surface shape.

#### <Formation of First Electrode 26 and Second Electrode 28>

A conductive copper tape having a width of 12.5 mm and a length of 70 mm (a first copper tape 48a, No. 8701 available from Sliontec Corporation, throughout Examples) was attached to each of the opposite ends of the transparent film 40 having the curved surface shape. The first copper tapes 48a were arranged approximately parallel to each other. A conductive copper tape having a width of 15 mm and a length of 25 mm (a second copper tape 48b) was further arranged in the direction perpendicular to each first copper tape 48a. The second copper tapes 48b were partially overlapped with the

first copper tapes 48a. Thus, a pair of electrodes (a first electrode 26 and a second electrode 28) were formed.

#### <Cutting Treatment: Production of Heat Generator 20>

As shown in FIG. 8, the periphery of the transparent film 40 having the curved surface shape, on which the mesh pattern 24, the first electrode 26, and the second electrode 28 were formed, was cut along a cutting line L1 corresponding to the formed shape while maintaining the first electrode 26 and the second electrode 28, to obtain a circular projected shape having a diameter of 110 mm. Furthermore, 20-mm curved portions at the ends were cut along cutting lines L2 and L3 while maintaining the first electrode 26 and the second electrode 28. Thus, as shown in FIG. 9, a heat generator 20A having a curved surface shape was produced. The heat generator 20A had an approximately rectangular projected shape, and had the first electrode 26 and the second electrode 28 on the short sides.

#### <Injection Forming: Production of Front Cover 10>

As shown in FIG. 14, the heat generator 20 having the curved surface shape was placed in an injection mold 50 for forming a front cover 10, and a polycarbonate melted at 300° C. was introduced into a cavity 52 thereof. Thus, as shown in FIG. 19, a front cover 10A according to Example 1 having a thickness of 2 mm was produced. The injection mold 50 was used under a temperature of 95° C. and a forming cycle of 60 seconds.

#### Reference Example 1

A transparent film 40 having a curved surface shape was prepared in the same manner as Example 1. Then, instead of the conductive copper tapes (the first copper tapes 48a) having a width of 12.5 mm and a length of 70 mm, conductive copper tapes 102 were attached to the opposite circumference portions to form a first electrode 26 and a second electrode 28 having an arc shape with a length of approximately 80 mm. A heat generator 200A having a circular projected shape was produced without cutting the end curved portions of the transparent film 40, and was insert-formed. Thus, as shown in FIG. 20, a front cover 100A according to Reference Example 1 was produced.

#### (Evaluation)

In each front cover, the minimum value Lmin and the maximum value Lmax of the distance between the first electrode 26 and the second electrode 28 (the electrode distance) were measured, and the parameter Pm was obtained using the following expression:

$$Pm = (L_{max} - L_{min}) / ((L_{max} + L_{min}) / 2).$$

As shown in FIG. 19, in Example 1, the maximum value Lmax of the distance between the electrodes was the length of an arc between points Ta and Ta' (shown by a dashed-dotted line, protruded forward in the drawing, throughout Examples), and the minimum value Lmin of the electrode distance was the length of an arc between points Tb and Tb'. The front cover 10A of Example 1 had a maximum value Lmax of 70 mm and a minimum value Lmin of 66 mm, and thus had a parameter Pm of 0.059 obtained using the above expression.

On the other hand, as shown in FIG. 20, in Reference Example 1, the maximum value Lmax of the distance between the electrodes was the length of an arc between points Tc and Tc', and the minimum value Lmin of the electrode distance was the length of an arc between points Td and Td'. The front cover 100A of Reference Example 1 had a

maximum value Lmax of 105 mm and a minimum value Lmin of 50 mm, and thus had a parameter Pm of 0.710 obtained using the above expression.

In each of the front cover 10A of Example 1 and the front cover 100A of Reference Example 1, a direct voltage was applied between the first electrode 26 and the second electrode 28. After the voltage was applied for 10 minutes, the cover surface temperatures were measured by an infrared thermometer to evaluate the temperature distribution. The measurement was carried out at the room temperature of 20° C. The results of the temperature distribution measurement are shown in FIGS. 21 and 22, and the measured temperatures (the minimum and maximum temperatures) and the temperature rises (the minimum, maximum, and average rises) are shown in Table 1. The temperature distribution of Example 1 is shown in FIG. 21, and that of Reference Example 1 is shown in FIG. 22.

TABLE 1

|           | Measured temperature (° C.) |         |            | Temperature rise (° C.) |         |         | Electrode distance (mm) |      |       |
|-----------|-----------------------------|---------|------------|-------------------------|---------|---------|-------------------------|------|-------|
|           | Minimum                     | Maximum | Difference | Minimum                 | Maximum | Average | Lmax                    | Lmin | Pm    |
| Example 1 | 33                          | 38      | 5          | 13                      | 18      | 15.5    | 70                      | 66   | 0.059 |
| Reference | 33                          | 53      | 20         | 13                      | 33      | 23.0    | 105                     | 50   | 0.710 |
| Example 1 |                             |         |            |                         |         |         |                         |      |       |

The front cover 10A of Example 1 exhibited a difference of approximately 5° C. between the minimum and maximum temperatures, a minimum temperature rise of 13° C., a maximum temperature rise of 18° C., and an average temperature rise of 15.5° C. In Example 1, the energy could be reduced by 2.5° C. as compared with an example requiring a temperature rise of 18° C. on average, thereby being advantageous in energy saving. In addition, as shown in FIG. 21, the heat generation was uniformly caused in the entire heat generator.

In contrast with Example 1, the front cover 100A of Reference Example 1 exhibited a larger difference of 20° C. between the minimum and maximum temperatures, a larger average temperature rise of 23.0° C., a minimum temperature rise of 13° C., a maximum temperature rise of 33° C., and a significantly larger variation. In addition, as shown in the temperature distribution of FIG. 22, the heat generation was caused only in the vicinity of the ends of the first and second electrodes and was hardly caused in the center.

As is clear from the above results, the heat generator of Example 1 satisfying the inequality of  $Pm \leq 0.375$  exhibited uniform heat generation on the entire surface, unlike the heat generator of Reference Example 1 not satisfying the inequality.

#### Second Example

In each of front covers of Examples 2 to 5 and Reference Example 2, the difference between the minimum and maximum temperatures was measured. In Examples 2 to 5 and Reference Example 2, a transparent film 40 having a mesh pattern 24 was formed under vacuum using a forming mold 42 (see FIGS. 6A and 6B) in the same manner as in Example 1. The forming mold 42 had a diameter of 173 mm and a shape provided by cutting off a part of a sphere having a radius of 100 mm. As shown in FIG. 10, the periphery of the transparent film 40 having the curved surface shape was cut along a cutting line L1 corresponding to the formed shape to obtain a circular projected shape, and curved portions 41 at the ends are cut along cutting lines L2 and L3. Thus, as shown in FIG.

23, transparent films 40 according to Examples 2 to 5 and Reference Example 2 were prepared. The width W was 60 mm in Example 2, 80 mm in Example 3, 90 mm in Example 4, 110 mm in Example 5, and 130 mm in Reference Example 2.

Then, as shown in FIG. 23, conductive copper tapes having a width of 15 mm (first copper tapes 48a) were attached to the opposite circumference portions of the transparent film 40 to form a first electrode 26 and a second electrode 28. Thus obtained heat generator was subjected to an injection forming in the same manner as Example 1, whereby heater-integrated-type front covers according to Examples 2 to 5 and Reference Example 2 were produced respectively.

(Evaluation)

Also in each of the front covers, the minimum value Lmin and the maximum value Lmax of the distance between the first electrode 26 and the second electrode 28 (the electrode

distance) were measured, and the parameter Pm was obtained using the following expression:

$$Pm = (Lmax - Lmin) / ((Lmax + Lmin) / 2).$$

As shown in FIG. 23, in Examples 2 to 5 and Reference Example 2, the maximum value Lmax of the electrode distance was the length of an arc between points Te and Te' (protruded forward in the drawing, throughout Examples), and the minimum value Lmin of the electrode distance was the length of an arc between points Tf and Tf'. The maximum value Lmax, the minimum value Lmin, and the parameter Pm in each of Examples 2 to 5 and Reference Example 2 are shown in the right of Table 2.

In each of the front covers of Examples 2 to 5 and Reference Example 2, a direct voltage was applied between the first electrode 26 and the second electrode 28. After the voltage was applied for 10 minutes, the cover surface temperatures were measured by an infrared thermometer to evaluate the temperature distribution. The measurement was carried out at the room temperature of 20° C. The measured temperatures (the minimum temperature, the maximum temperature, and the difference thereof) are shown in the left of Table 2.

TABLE 2

|           | Measured temperature (° C.) |         |            | Electrode distance (mm) |      |       |
|-----------|-----------------------------|---------|------------|-------------------------|------|-------|
|           | Minimum                     | Maximum | Difference | Lmax                    | Lmin | Pm    |
| Example 2 | 34                          | 39      | 5          | 209                     | 194  | 0.074 |
| Example 3 | 32                          | 38      | 6          | 209                     | 182  | 0.139 |
| Example 4 | 31                          | 39      | 8          | 209                     | 174  | 0.182 |
| Example 5 | 26                          | 38      | 12         | 209                     | 155  | 0.298 |
| Reference | 24                          | 40      | 16         | 209                     | 130  | 0.471 |
| Example 2 |                             |         |            |                         |      |       |

Each front cover of Examples 2 to 4 exhibited a difference of approximately 5° C. to 8° C., and the front cover of Example 5 exhibited a difference of approximately 12° C., between the minimum and maximum temperatures. Thus, the

## 21

front covers of Examples 2 to 5 exhibited uniform heat generation on the entire surfaces, thereby being advantageous in energy saving. In contrast, the front cover of Reference Example 2 exhibited a difference of 16° C., and the heat generation was not uniformly caused on the entire heat generator.

As is clear from the above results, the heat generators of Examples 2 to 5 satisfying the inequality of  $P_m \leq 0.375$  exhibited uniform heat generation on the entire surfaces, unlike the heat generator of Reference Example 2 not satisfying the inequality.

It is to be understood that the car light front cover, the front cover production method, and the electric heating structure of the present invention are not limited to the above embodiments, and various changes and modifications may be made therein without departing from the scope of the present invention.

The invention claimed is:

1. A car light front cover, which is attached to a front opening of a car light having a lamp body and a light source disposed in the lamp body, wherein

the front cover comprises a heat generator having a three-dimensional curved surface disposed in a part facing the light source, and

the heat generator has a mesh pattern containing a conductive thin metal wire with a plurality of lattice intersections, and has a first electrode and a second electrode formed on opposite ends of the mesh pattern.

2. A car light front cover according to claim 1, wherein the thin metal wire in the mesh pattern has a width of 1 to 40  $\mu\text{m}$ .

3. A car light front cover according to claim 1, wherein the thin metal wire in the mesh pattern has a pitch of 0.1 to 50 mm.

4. A car light front cover according to claim 1, wherein when two opposite points in the first electrode and the second electrode are at a distance,  $L_{min}$  is a minimum value of the distance, and  $L_{max}$  is a maximum value of the distance, the first electrode and the second electrode satisfy an inequality:

$$(L_{max}-L_{min})/((L_{max}+L_{min})/2) \leq 0.375.$$

5. A car light front cover according to claim 1, wherein the thin metal wire in the mesh pattern has a metallic silver portion formed by exposing and developing a silver salt-containing layer containing a silver halide.

6. A car light front cover according to claim 1, wherein the heat generator has a surface resistance of 10 to 500 ohm/sq.

7. A car light front cover according to claim 1, wherein the heat generator has an electrical resistance of 12 to 120 ohm.

8. A car light front cover according to claim 1, wherein the three-dimensional curved surface of the heat generator has a minimum curvature radius of 300 mm or less.

## 22

9. A method for producing a car light front cover, which is attached to a front opening of a car light having a lamp body and a light source disposed in the lamp body, wherein

the front cover comprises a heat generator disposed in a part facing the light source,

the method comprises a heat generator preparation process of preparing the heat generator and an injection process of placing the heat generator in a mold and then injecting a melted resin into the mold, and

the heat generator preparation process contains a pattern formation step of forming a mesh pattern containing a conductive thin metal wire with a plurality of lattice intersections on an insulating transparent film, a shape forming step of forming the transparent film into a three-dimensional curved surface corresponding to a surface shape of the front cover,

an electrode formation step of forming a first electrode and a second electrode on the opposite ends of the transparent film, and

a cutting step of cutting a part of the transparent film having the three-dimensional curved surface.

10. A method according to claim 9, wherein the thin metal wire formed in the pattern formation step has a width of 1 to 40  $\mu\text{m}$ .

11. A method according to claim 9, wherein the first electrode and the second electrode are formed in the electrode formation step such that when two opposite points in the first electrode and the second electrode are at a distance,  $L_{min}$  is a minimum value of the distance, and  $L_{max}$  is a maximum value of the distance, the first electrode and the second electrode satisfy an inequality:

$$(L_{max}-L_{min})/((L_{max}+L_{min})/2) \leq 0.375.$$

12. A method according to claim 9, wherein the mesh pattern containing the thin metal wire is formed in the pattern formation step such that the thin metal wire has a metallic silver portion formed by exposing and developing a silver salt-containing layer containing a silver halide disposed on the transparent film.

13. A method according to claim 9, wherein the heat generator has a three-dimensional curved surface with a minimum curvature radius of 300 mm or less.

14. An electric heating structure comprising a heat generator having a three-dimensional curved surface, wherein the heat generator has a mesh pattern containing a conductive thin metal wire with a plurality of lattice intersections, and has a first electrode and a second electrode formed on opposite ends of the mesh pattern.

\* \* \* \* \*